

Jan. 29, 1952

E. H. LAND  
PHOTOGRAPHIC SILVER TRANSFER PRODUCT  
AND PROCESS, INCLUDING A LEAD SALT  
Filed April 13, 1946

2,584,029

FIG. 1



FIG. 2



*Edwin H. Land*  
INVENTOR

BY *Donald R. Brown*  
ATTORNEY

## UNITED STATES PATENT OFFICE

2,584,029

## PHOTOGRAPHIC SILVER TRANSFER PRODUCT AND PROCESS, INCLUDING A LEAD SALT

Edwin H. Land, Cambridge, Mass., assignor to Polaroid Corporation, Cambridge, Mass., a corporation of Delaware

Application April 13, 1946, Serial No. 662,000

29 Claims. (Cl. 95—8)

1

This invention relates to photography and more particularly to novel photographic film units and materials, and methods for utilizing such film units and materials.

More specifically, a preferred form of the present invention relates to improvements over the novel photographic film units and processes disclosed in my copending application Serial No. 576,254 filed February 5, 1945, for Photographic Process, Apparatus and Product, now abandoned. It is, however, not limited to use with such processes or films.

The principal object of the present invention is to provide photographic materials and processes which enable the production of a positive image having increased contrast, gamma and stability.

Another object of the invention is to provide a photographic image having a pH varying in accordance with the density of said image, said pH being high in the shadows and low in the highlights.

Another object of the invention is to provide a composite photographic film unit comprising a photosensitive layer, an image-carrying layer and a container having therein a liquid composition, said liquid composition comprising a solvent for a developer and an alkali, said film unit having therein a developer and an alkali, said image-carrying layer having associated therewith a substance capable of reducing the alkalinity of said image-carrying layer when said liquid composition is spread in contact therewith.

Another object of the invention is to provide in a photographic process of the type wherein a layer of photosensitive material is treated with a liquid composition, including a developer, and a positive image is created by transferring image-forming components from said layer to another layer, the improvement which comprises increasing the contrast and gamma of said image by forming said image in the presence of a substance capable of reducing the alkalinity of said image in the highlights thereof.

A still further object of the invention is to provide a photographic process which comprises treating a layer of exposed photosensitive material with an alkaline liquid composition containing a developer, an alkali, and a substance capable of forming image-forming components with undeveloped portions of said photosensitive material, transferring said image-forming components to another layer and creating on said other layer a positive image having dense blacks and clear highlights by reacting said image-forming

2

components with said alkaline liquid composition and preventing the oxidation of any excess developer in the area of said highlights by reducing the alkalinity of said liquid composition in the area of said highlights to a point where oxidation of said developer does not occur.

A still further object of the invention is to provide a photographic sheet material capable of acting as a carrier for a final positive image when formed into a permeable assembly with an undeveloped exposed photosensitive layer and permeated with a liquid composition containing a solvent, a developer, a material for forming positive image-forming components and a film-forming material, said sheet material having associated therewith a substance capable of reacting with said film-forming material to form therewith compounds less soluble in water than said film-forming material.

20 These and other objects of the invention will in part be obvious and will in part appear hereinafter.

In one form of the present invention there is provided a composite photographic film unit 25 having a photosensitive layer and another layer. The other layer may serve several functions. In a preferred example it acts as a backing layer to permit the spreading of a liquid composition in a layer parallel to the photosensitive layer and it 30 also performs the additional function of serving as a carrier for the final positive image. In less preferred forms of the invention it serves only either one of these functions or merely acts to carry certain of the reactive ingredients. In al- 35 most all cases, however, it will have the additional function of forming, with the photosensitive layer, a unit only slowly permeable to oxygen and within which a photographic reaction may take place with substantial freedom from the effects 40 of aerial oxidation. This layer is referred to as an image-carrying layer. Between these two layers there is included a rupturable container or pod having therein a liquid composition. This composition is preferably viscous, preferably 45 alkaline and preferably contains therein a developer and a film-forming material. The liquid composition also preferably contains a substance which will react with the unexposed portions of the photosensitive layer to form therewith soluble image-forming complexes. When the pod is 50 ruptured and the viscous developing composition is spread between the photosensitive layer and the image-carrying layer, it forms an image-receiving layer. This layer is stabilized by the action of the film-forming substance which, dur-

ing the processing of the film, is converted from a fluid to a solid. The positive image-forming complexes are transferred from the photosensitive layer to the image-receiving layer, where the positive image is formed. The photosensitive layer is next preferably stripped from the image-receiving layer to reveal the finished positive image.

The present invention deals primarily with the improvement of the above process and product by increasing the stability, contrast and gamma of the resultant image and the insolubility and dimensional stability of the formed film. The present invention is not limited to use with the above product or process, however.

For a fuller understanding of the nature and objects of the invention reference should be had to the following detailed description taken in connection with the accompanying drawings, wherein:

Figure 1 is an exaggerated cross-sectional view of a preferred embodiment of the present invention; and

Fig. 2 is an exaggerated cross-sectional view of another embodiment of the present invention.

As shown in Fig. 1, there is provided a base layer 10 adapted to carry on one surface thereof of a photosensitive layer 11. There is also provided an image-carrying layer 12 which may be joined to the base layer 10 by means of a hinge 14. Between the image-carrying layer 12 and the photosensitive layer 11, there is positioned a container 13, adapted to have therein a liquid composition. This container can be attached to either the photosensitive layer 11 or the image-carrying layer 12. Films of this general character are described in my copending application mentioned above. On the upper surface of the image-carrying layer 12, there is preferably incorporated an insolubilizing agent whose function will be described in more detail later.

The base layer 10 is preferably made of a suitable film base material such as a cellulosic ester, or mixed ester such as cellulose nitrate, cellulose acetate, cellulose acetate propionate, or other substances capable of supporting a photosensitive emulsion.

This base can be made opaque, if desired, by the addition of suitable dyes or pigments to the above-named substances, or the base 10 can be made of paper and other materials suitable for supporting a photosensitive emulsion. Such opacity will be preferable depending upon how the film is exposed within the camera. It may also be made of an impermeable substance such as glass.

The photosensitive layer is preferably of the type rendered developable by exposure to light, e. g., an emulsion of a silver halide, or of a mixture of silver halides or of a mixed silver halide.

The image-carrying layer 12, in a preferred embodiment of the invention, is formed of a photographic material, known in the art as baryta paper, although it can be made of other substances. This layer is preferably permeable to a substance contained in the liquid composition and may also be manufactured from other substances such as gelatin or paper. It may also be made of gelatin, regenerated cellulose, poly-hydroxy alkanes such as polyvinyl alcohol, sodium alginate, certain of the cellulose ethers such as methyl cellulose, and their derivatives such as sodium carboxymethyl cellulose or hydroxyethyl cellulose, carbohydrates such as gums or starch, and mixtures of these materials where

the latter are compatible. It may, however, be made of relatively impermeable materials such as glass, Celluloid and other materials commonly used in the photographic arts.

The liquid composition, in its preferred embodiment, is composed of a developer such as hydroquinone, a film-forming substance such as sodium carboxymethyl cellulose, and a substance adapted to form from a latent photographic image a positive image-forming component. This latter substance in a preferred form of the invention is sodium thiosulfate. There are also preferably included other substances to aid the photographic reaction, such as a preservative, i. e. sodium sulfite, and an alkali, i. e. sodium hydroxide, plus water to carry the above-mentioned elements in solution. Suitable liquid compositions may be produced as shown in the following nonlimiting examples.

#### Example #1

The following substances are put in a beaker and stirred with a plastic rod until dissolved:

|                             |       |      |
|-----------------------------|-------|------|
| Water                       | cc    | 476  |
| Sodium sulfite (desiccated) | grams | 18   |
| Sodium hydroxide            | do    | 17.5 |

The following substance is then stirred into the above mixture with a plastic rod to avoid lumps: Sodium carboxymethyl cellulose, medium viscosity (Lot No. 1155 Hercules), 42.62 grams.

The above mixture is stirred in a closed mixer having a nitrogen atmosphere over the liquid therein, and the temperature is raised to 178° F. The mixture is maintained at this temperature for approximately 3½ hours. During the first two hours 10 grams of sodium thiosulfate are added to the above mixture. During the last hour of heat treatment 18 grams of hydroquinone are added to the mixture. 249 cc. of water are then added to the mixture sometime before the completion of the 3½ hour heating period.

#### Example #2

The following substances are put in a beaker and stirred with a plastic rod until dissolved:

|                             |       |       |
|-----------------------------|-------|-------|
| Water                       | cc    | 476   |
| Sodium sulfite (desiccated) | grams | 9     |
| Sodium hydroxide            | do    | 19.50 |

The following substance is then stirred into the above mixture with a plastic rod to avoid lumps: Sodium carboxymethyl cellulose, medium viscosity (Lot No. 1155 Hercules), 42.62 grams.

The above mixture is stirred in a closed mixer having a nitrogen atmosphere over the liquid therein, and the temperature is raised to 178° F. The mixture is maintained at this temperature for approximately 3½ hours. During the first two hours 2.5 grams of sodium thiosulfate are added to the above mixture. During the last hour of heat treatment 9 grams of hydroquinone are added to the mixture. 237 cc. of water are then added to the mixture sometime before the completion of the 3½ hour heating period.

Various equivalents may be used in the above-mentioned liquid composition and it is equally possible to substitute for the thickening and film-forming sodium carboxymethyl cellulose other film-forming agents, such as hydroxyethyl cellulose, or gelatin, or such materials as sodium alginate, or starch. Equally, other developers, preservatives and alkalies may be used, and other substances such as restrainers may be added.

In the use of the invention as described above, the photosensitive layer is exposed to actinic light

and, without further exposure to light, the whole assembly is subjected to a mechanical stress such as by passing through a wringer, not shown, starting with the hinge end 14. As the film is squeezed through the wringer, the container 13 is ruptured and the liquid composition is uniformly spread between the photosensitive layer 11 and the image-carrying layer 12.

When the liquid composition is spread between the photosensitive layer 11 and the image-carrying layer 12, the following reaction takes place: the developer develops the latent photographic image and the sodium thiosulfate dissolves the unexposed silver halide grains and carries them into the image-receiving layer, being formed by the solidification of the film-forming substance contained in the liquid composition. These unexposed silver halide grains are then developed and formed into a positive image. While this process is in operation as stated above, the film-forming substance, i. e. the sodium carboxymethyl cellulose, is being solidified into a dimensionally stable film.

It has been found that it is possible to substantially improve the products and processes described above by increasing the insolubility of the image-receiving layer, increasing the contrast of the positive image, increasing the gamma, increasing the density of the transferred image-forming components, and insolubilizing various unexhausted elements of the liquid composition.

The above can be accomplished by placing preferably within or upon the upper surface of the image-carrying layer 12 a material which enters into the photographic reaction to bring about the results set forth above. Of the materials which have been found satisfactory, those showing the most extraordinary results are generally the lead salts, and, of the lead salts, lead acetate appears to be the most desirable. In the preferred modification of the invention, image-carrying layer 12 is coated with a solution of a lead salt such as lead acetate, and the solvent is allowed to evaporate, leaving within and upon the surface of the layer 12 a precipitate of lead acetate. When the above-described photographic process is practiced and the liquid composition is spread between the photosensitive layer 11 and the lead acetate coated layer 12, the lead acetate is taken into solution by a solvent (water) in the liquid composition, and substantially improves and increases the contrast, gamma and stability of the final positive image. It whitens the highlights and increases the density of the shadows.

All of the reactions involved in this substantial improvement of the quality and stability of the final positive image are not completely understood, and in some cases, it is difficult to differentiate between cause and effect in the various reactions which are going on simultaneously. There are, however, certain reactions which can be set forth with a considerable degree of certainty. In the first place, it is quite definitely known that the lead acetate reacts with a polymeric substance such as sodium carboxymethyl cellulose to form cross-linkages therewith and thereby create a compound having an increased insolubility in water. This is believed to hasten the precipitation of the film-forming sodium carboxymethyl cellulose, thereby speeding up the formation of the image-receiving layer. The compound resulting from the interaction of the lead acetate and the sodium carboxymethyl cellulose gives a more dimensionally stable film, having an increased insolubility in water.

The lead acetate remarkably increases the contrast and gamma of the positive image produced in the image-receiving layer, although it is not completely understood how this effect is accomplished. There are certain observed conditions which would explain this improvement of the positive image, but the reason for the existence of these conditions is not readily ascertainable from a theoretical analysis of the various reactions. The positive image formed in the presence of lead acetate has very much denser blacks than a positive image formed under exactly the same circumstances wherein lead acetate is not used. This intensification of blacks is believed to be caused by an increase in the amount and size of the silver grains forming the positive image. A remarkable increase in intensification is provided by the use of lead salts generally and lead acetate in particular. It is believed that the lead reaction with the sodium carboxymethyl cellulose changes the character of the film being formed to such an extent that the silver formed therein is formed in larger grain sizes, whereby a greater density is achieved, and less scattering of light results.

It has also been observed that an image produced without the use of a material such as lead acetate has a more or less overall uniform alkalinity; while an image produced with the use of lead acetate has a remarkable variation in pH from point to point, and it has been found that those images having the clearest whites and the darkest blacks showed a condition which was slightly acid or neutral, i. e. a pH of 6-8, in the highlights and quite basic, i. e. a pH of above 9, in the shadows. It is believed that this slightly acid or neutral condition plays an extremely important part in at least the preservation of clear whites. One of the reasons for believing this is that those images, lacking clear highlights, are apparently stained by an oxidation product of the developer. Such a stain is eliminated when lead acetate is used in sufficient quantity to convert the highlights to a slightly acid or neutral condition. It is believed that this is due to the fact that the developer is incapable of being oxidized in a neutral or slightly acid solution. Therefore, no stain can form even though a potential stain-forming component exists in the whites which is made inactive by the lower pH. The presence of this stain-forming component in the highlights has been experimentally ascertained by taking a positive image, having clear highlights, produced with a lead acetate-coated image-carrying layer and placing a drop of sodium hydroxide on a clear highlight. This sodium hydroxide raises the pH considerably and a brown stain appears.

In the preferred form of the invention, lead acetate is used as the insolubilizing agent. This lead salt seems to be particularly efficient for accomplishing the results mentioned above and is quite easily usable since it is soluble in water.

A preferred method of incorporating the lead acetate in the image-carrying layer 12 is as follows:

1575 grams of lead acetate are dissolved in 3500 cc. of water. This mixture is placed in a shallow container and heated to approximately 80-90° F. A continuous roll of double-weight baryta paper is then passed over the lead acetate bath for approximately two minutes. The paper is suspended near the bath by rollers in such a way that only one surface thereof will contact the bath. Thus, only one surface is coated. After passing through the bath, the paper is passed

over a drying drum which is heated to approximately 75-90° F. The coated surface of the paper is in contact with the drum for approximately 7½ minutes. This is a preferred method of coating lead acetate upon double-weight baryta paper, but other methods may equally be used.

This method of coating the baryta paper is preferred since it places the poisonous lead acetate on the inner surface only of the image-carrying layer. Thus, in the handling of the film pack the fingers of a user do not contact the lead-acetate-coated surface. Of course, when the film unit has been processed in the manner described above, the lead has combined with the materials used and has formed insoluble salts.

Despite the formation of these insoluble salts, it is strongly recommended that care be used in handling the finished picture, lest some soluble lead salts remain. The finished picture should not be placed in the mouth.

In view of the fact that lead salts are highly poisonous, another preferred form of the present invention embodies the use of a lead salt which is insoluble in water. As an example of this, there is used lead tartrate which is deposited upon and within the surface of the image-carrying layer 12. With lead tartrate used in place of a water-soluble lead salt, such as lead acetate, the lead tartrate will not normally be removed from the layer 12 by handling. For instance, it will not be picked up by the fingers of a user when he touches the surface of the base, since the lead tartrate will not be dissolved by the perspiration normally on the surface of the skin. When the liquid composition is spread between the photosensitive layer and the support layer containing the lead tartrate, the lead tartrate is dissolved by a solvent therefor and subsequently performs all, or substantially all, of the reactions attributable to lead acetate.

In this connection, it has been found that the liquid compositions set forth in the previous examples have a solvent effect on lead tartrate, although this lead salt is insoluble in water. It is believed that this effect is due to the sodium hydroxide which apparently dissolves the lead tartrate and forms therewith insoluble compounds more slowly than the other elements of the combination; thus the lead is in ionic condition for reaction with the other elements of the composition.

Numerous other lead salts, such as lead nitrate, lead bromide, lead chlorate, lead perchlorate, lead citrate, lead isobutyrate, lead peroxydisulfate, or lead dithionate may be used in the practice of the present invention. The lead salts may be used singly or jointly; for example, excellent results have been obtained with an image-carrying layer first coated with lead acetate and then with lead nitrate.

Since lead salts are extremely poisonous, persons working with these salts should utilize the normal precautions practiced with any use of lead salts.

Some of these lead salts are insoluble in water but soluble in other substances. If those solvents are not normally included in the liquid composition, they are added so that the liquid composition will dissolve the lead salt. If it is undesirable to include this solvent in combination with the other elements of the liquid composition for too long a time, a separate container is included to carry the solvent.

Zinc acetate may also be used for whitening

the highlights. This material may be placed within and upon the surface of the image-carrying layer 12 in the same manner as practiced with the lead salts. The zinc acetate is also taken into solution by a solvent therefor contained in the liquid composition and reacts in much the same way, except that it does not insolubilize the sodium carboxymethyl cellulose. It does, however, whiten the highlights.

It is believed that the beneficial results obtained with the zinc acetate are due partly to its ability to reduce the alkalinity in the neighborhood of the highlights of the positive image.

It has also been found that it is possible to practice the present invention by incorporating an agent such as a lead salt in or upon the lower surface of the photosensitive layer. In this instance, the operation is the same end, and as the liquid composition is spread between the photosensitive layer and the image support layer, it dissolves the lead salt from the photosensitive layer and the lead salt acts in the same manner as described above.

When the lead salt is carried by the photosensitive layer, precautions should be taken to insure that the lead salt is in a stratum separate from the photosensitive material since the lead salts appear to have a strong desensitizing effect on the photosensitive material.

It is also practicable to carry the agent, such as a lead salt, out of contact with either the photosensitive layer or the support layer.

Since the lead salt has a coagulating effect upon some of the film-forming materials used in the present invention, it is preferred in this embodiment of the invention to have the lead salt and a solvent therefor contained in a separate container or pod. A means for accomplishing this result is shown in Fig. 2 where like numbers correspond to like numbers in Fig. 1. As shown here, a separate container 15 may be placed immediately adjacent the container 13 carrying the liquid composition. Thus, when the film is exposed and processed by running through a wringer, the lead salt solution is released and is spread, along with the liquid composition, between the photosensitive layer and the image-carrying layer.

In those cases where a film-forming substance is used which is not hardened by a lead salt, the lead salt has the ability to increase the contrast and gamma of the final positive, even though it may not insolubilize any formed film. Examples of such film-forming materials are hydroxyethyl cellulose and polyvinyl alcohol.

In some instances it is desirable to practice the present invention without the use of a film-forming material. If such be the case, the photographic process is substantially the same as that described above and the final positive image is formed on and within the surface of the image-carrying layer. In such a modification of the invention, the lead salts have a very beneficial effect upon the final image, increasing its stability, contrast and gamma. Zinc acetate similarly increases the clearness of the highlights when used with a liquid composition having no film-forming material.

Another, though less preferred, method of practicing the present invention is to have certain of the materials which are preferably included in the liquid composition placed elsewhere in the film unit. For instance, it is possible to deposit the developer and hypo in solid form on the image-carrying layer. In this

case, the container might have therein only water or an aqueous solution of sodium carboxymethyl cellulose.

It is also possible to extrude a sheet of sodium carboxymethyl cellulose containing therein, in solid form all of the materials ordinarily dissolved in the water in the liquid container. This sheet can be placed between the photosensitive layer 11 and the image-carrying layer 12. The layer 12 has thereon an insolubilizing agent such as lead acetate. In this modification of the invention, the container has only therein a solvent, such as water, for the various materials incorporated into the extruded sheet. When the water is spread in contact with this extruded sheet, it dissolves the sheet and the remainder of the process is the same as that discussed in connection with Fig. 1.

One advantage of this last-mentioned modification is that it eliminates the necessity for a liquid container and in this case the film unit may be processed by merely wetting it in a water bath until a sufficient amount of water has been absorbed by the film unit to give the desired concentrated solution of the reactive materials.

It is equally possible to place such an extruded sheet between the base layer 10 and the photosensitive layer 11, although in this latter case it is desirable to include an additional film-forming material within the water carried by the container, since it is desirable to form the final positive image in a film created during the process.

It should also be understood that, although the invention has been described in terms of individual film units, it may be practiced with roll films wherein a plurality of images are produced and the roll film may be treated so as to produce each image separately or all images simultaneously.

The use of soluble lead salts, and specifically lead acetate, in silver halide transfer processes is also disclosed in certain other of my copending applications, such, for example, as Serial No. 700,931, filed October 3, 1946, for Photographic Product and Process, and Serial No. 708,007, filed November 6, 1946, for Photographic Product and Process.

Since certain changes in carrying out the above process, and certain modifications in the article which embody the invention may be made without departing from its scope, it is intended that all matter contained in the above description or shown in the accompanying drawings shall be interpreted as illustrative and not in a limiting sense.

What is claimed is:

1. A photographic product comprising a photographic product comprising a photosensitive material which includes a silver halide layer, a base layer for receiving, by transfer, a positive print, and a rupturable containing means holding a liquid, said product having positioned therein photographic reagents including a silver halide developer, a silver halide solvent and a lead salt soluble in said liquid, said containing means and said layers being so held together that said containing means is capable, upon rupture, of releasing at least part of its contents to permeate superposed portions of said photosensitive layer and said base layer, said liquid, upon release, rendering said silver halide developer and said silver halide solvent effective to develop a latent image in said photosensitive layer and to form soluble silver com-

plexes with the undeveloped silver halide of said photosensitive layer and, additionally, providing a solution of the lead salt adjacent the surface of the print-receiving area of said base layer in which part at least of the soluble silver complex is reduced to silver to produce the positive print.

2. The product of claim 1 wherein the liquid is a dispersion of a film-forming organic colloid, and the lead salt is capable of reacting with said colloid to give a reaction product less soluble in said liquid than said colloid.

3. The product of claim 1 wherein the lead salt is lead acetate.

15 4. The product of claim 1 wherein the lead salt is lead tartrate.

5. The product of claim 1 wherein the containing means comprises a single elongated enclosure which contains all of said liquid, and 20 an elongated dispensing lip which parallels said enclosure and is rupturable to provide a passage for said liquid.

6. The product of claim 1 wherein the containing means comprises a pair of liquid-containing enclosures, each including a rupturable liquid-dispensing lip for providing a passage therefrom to said image-receiving area, the liquid in one of said enclosures comprising a dispersion of the silver halide solvent and the 25 silver halide developer, and the liquid in the other of said enclosures comprising a dispersion of the lead salt.

7. The product of claim 6 wherein the dispersions are solutions.

35 8. A photographic product comprising a photosensitive silver halide layer, a base layer, and a rupturable container holding a liquid, said layers and said container being attached together so as to permit said layers to be superposed with said container so positioned as to release its liquid for spreading in a film between said layers, the liquid in said container comprising a silver halide developer, a silver halide solvent and an organic film-forming colloid, said 40 base layer having dispersed therein a lead salt soluble at least in part in said liquid.

9. The product of claim 8 wherein the lead salt is located adjacent only that surface of said base layer which adjoins said photosensitive layer when said layers are superposed.

10. The product of claim 8 wherein the solution is an aqueous solution and the organic film-forming colloid dissolved therein is sodium carboxymethyl cellulose, and the sheet support is 45 baryta paper.

55 11. The product of claim 10 wherein the aqueous solution includes hydroquinone, sodium thiosulfate and sodium hydroxide, and the lead salt is lead acetate.

12. A photographic product capable of forming transfer prints in conjunction with a photosensitive silver halide element, said product comprising a rupturable containing means holding a liquid and a sheet support upon which said containing means is mounted, said sheet support providing an image-receiving area adjacent said containing means onto which said liquid is spreadable in a thin layer directly from said containing means, said product carrying a silver halide developer, a silver halide solvent and a lead salt soluble in part at least in said liquid, said reagents and said liquid being sufficient in amount and being so located in relation to said image-receiving area that the spreading of said liquid over said area disperses silver halide de-

developer, silver halide solvent and lead salt throughout said area in adequate quantity to form a transfer print of a latent image in an area of a contiguous silver halide element equivalent to said image-receiving area.

13. The product of claim 12 wherein the liquid is a dispersion of a film-forming organic colloid, and the lead salt is capable of reacting with said colloid to give a reaction product less soluble in said liquid than said colloid.

14. The product of claim 12 wherein the lead salt is lead acetate.

15. The product of claim 12 wherein the lead salt is lead tartrate.

16. The product of claim 12 wherein the containing means comprises a single elongated enclosure which contains all of said liquid, and an elongated dispensing lip which parallels said enclosure and is rupturable to provide a passage for said liquid.

17. The product of claim 12 wherein the containing means comprises a pair of liquid-containing enclosures, each including a rupturable liquid-dispensing lip for providing a passage therefrom to said image-receiving area, the liquid in one of said enclosures comprising a dispersion of the silver halide solvent and the silver halide developer, and the liquid in the other of said enclosures comprising a dispersion of the lead salt.

18. The product of claim 17 wherein the dispersions are solutions.

19. A photographic product capable of forming transfer prints in conjunction with a photo-sensitive silver halide element, said product comprising a rupturable containing means holding an alkaline liquid solution of a silver halide developer, a silver halide solvent and an organic film-forming colloid, and a sheet support upon which said containing means is mounted, said sheet support providing an image-receiving area adjacent said containing means onto which said liquid solution is spreadable in a thin layer directly from said containing means, said support having distributed, at least throughout said image-receiving area, a lead salt soluble in said solution, said solution and said lead salt being sufficient in amount so that the spreading of said liquid over said area provides a dispersion of silver halide developer, silver halide solvent and lead salt throughout said area in adequate quantity to form a transfer print of a latent image in an area of a contiguous silver halide element equivalent to said image-receiving area.

20. The product of claim 19 wherein the lead salt is located adjacent only that surface of said support upon which the contents of the containing means are spread.

21. The product of claim 19 wherein the solution is an aqueous solution and the organic film-forming colloid dissolved therein is sodium carboxymethyl cellulose and the sheet support is baryta paper.

22. The product of claim 21 wherein the aqueous solution includes hydroquinone, sodium thiosulfate and sodium hydroxide, and the lead salt is lead acetate.

23. The process of forming positive images in silver which comprises developing a latent negative image in a silver halide emulsion layer with a solution comprising a silver halide developer and a silver halide solvent to form an imagewise distribution of soluble silver complex in said emulsion layer, transferring from said emulsion layer by imbibition at least part of

said imagewise distribution of said soluble silver complex to an image-carrying layer so superposed adjacent said emulsion layer as to receive a depthwise diffusion of said solution from said emulsion layer without appreciably disturbing the imagewise distribution of the silver complex in said solution, and reducing to silver the silver ions of said soluble silver complex in the presence of a lead salt soluble in said solution to form an image in silver which is a positive of the subject matter of said latent image.

24. The process of claim 23 wherein the lead salt is carried in solid form by said image-carrying layer in a position to be dissolved in the solution.

25. The process of claim 24 wherein the lead salt is dispersed adjacent only the surface of said image-carrying layer adjacent the photo-sensitive layer.

26. The process of claim 23 wherein a liquid containing an organic film-forming colloid is spread in a layer generally parallel to and adjacent the photosensitive emulsion in a position to permeate said emulsion and provides the liquid for the solution of the silver halide developer and the silver halide solvent.

27. The process of claim 26 wherein the liquid is spread between the silver halide emulsion layer and the image-carrying layer, and the lead salt reacts with the film-forming colloid in the liquid layer to form therewith a reaction product more insoluble in the liquid than the colloid.

28. The process of claim 27 wherein the lead salt is lead acetate.

29. A photographic product capable of forming transfer prints in conjunction with a photo-sensitive silver halide element, said product comprising a rupturable containing means holding a liquid and a sheet support upon which said containing means is mounted, said sheet support providing an image-receiving area adjacent said containing means onto which said liquid is spreadable in a thin layer directly from said containing means, said product carrying a lead salt soluble in part at least in said liquid and also at least one substance from the class consisting of the silver halide developers and the silver halide solvents, said liquid being sufficient in amount and being so located in relation to said image-receiving area that the spreading of said liquid over said area disperses said substance and lead salt throughout said area in adequate quantity to participate in the formation of a transfer print of a latent image in an area of a contiguous silver halide element equivalent to said image-receiving area.

EDWIN H. LAND.

#### REFERENCES CITED

The following references are of record in the file of this patent:

#### UNITED STATES PATENTS

| Number    | Name     | Date          |
|-----------|----------|---------------|
| 312,954   | Blain    | Feb. 24, 1885 |
| 1,610,783 | Jelley   | Dec. 14, 1926 |
| 1,916,350 | Wendt    | July 4, 1933  |
| 1,963,707 | LeJeune  | June 19, 1934 |
| 2,091,689 | Russell  | Aug. 31, 1937 |
| 2,217,189 | Sus.     | Oct. 8, 1940  |
| 2,224,269 | McIntosh | Dec. 10, 1940 |

13

## UNITED STATES PATENTS

| Number    | Name     | Date          |
|-----------|----------|---------------|
| 2,224,654 | McIntosh | Dec. 10, 1940 |
| 2,322,005 | Fierke   | June 15, 1943 |
| 2,322,006 | Fierke   | June 15, 1943 |
| 2,322,027 | Jelley   | June 15, 1943 |
| 2,352,014 | Rott     | June 20, 1944 |
| 2,355,884 | McIntosh | Aug. 15, 1944 |

## FOREIGN PATENTS

| Number            | Country       | Date          |
|-------------------|---------------|---------------|
| 12,678<br>of 1899 | Great Britain | July 22, 1899 |
| 10,051            | Great Britain | Apr. 30, 1906 |
| 24,667            | Great Britain | 1906          |
| 13,835            | Great Britain | 1907          |

14

| Number  | Country       | Date          |
|---------|---------------|---------------|
| 328,762 | Great Britain | May 8, 1930   |
| 372,637 | Great Britain | May 12, 1932  |
| 391,790 | Great Britain | May 3, 1933   |
| 413,853 | Great Britain | July 26, 1934 |
| 879,995 | France        | Mar. 10, 1943 |

## OTHER REFERENCES

|                                             |    |                                                |
|---------------------------------------------|----|------------------------------------------------|
| Beveridge: "Paper Makers Pocket Book," D.   | 10 | Van Nostrand & Company, 1925, page 238 cited.  |
| Wall: Intensification and Reduction, Ameri- |    | can Photographic Publishing Co., 1927, page 15 |
| cited (40 pp.).                             |    | cited (40 pp.).                                |

Clerc: Photography Theory and Practice, Pitman Publishing Co., pages 355-7 cited 2d edition, 1937.